

[54] ELEMENT HAVING BIMETAL PROPERTIES

3,107,532 10/1963 Lingnau ..... 73/363.5

[75] Inventors: **Friedrich Schneider; Dieter Stockel,**  
both of Pforzheim, Germany

Primary Examiner—Donald O. Woodiel  
Attorney, Agent, or Firm—Wenderoth, Lind & Ponack

[73] Assignee: **G. Rau**, Pforzheim, Germany

[22] Filed: **June 26, 1972**

[57] ABSTRACT

[21] Appl. No.: **266,351**

[30] Foreign Application Priority Data

July 20, 1971 Germany ..... 2136171

[52] U.S. Cl. ..... 73/363.5

[51] Int. Cl. ..... G01k 5/62

[58] Field of Search. .... 73/363.5, 363, 363.1;  
29/195.5, 191.6

[56] References Cited

UNITED STATES PATENTS

1,653,378 12/1927 Steel ..... 29/195.5

The subject of this invention is an element having bimetal properties and made of a composite fiber material comprising a matrix material and at least one group of fibers embedded therein. The bimetal properties may be achieved by using a matrix material having a coefficient of thermal expansion differing from that of at least one group of embedded fibers. Alternatively, the coefficients of thermal expansion of at least two groups of embedded fibers may differ from each other to achieve such properties. Yet another possibility is to combine these two methods to achieve the desired bimetal properties.

10 Claims, 3 Drawing Figures



Fig. 1



Fig. 2



Fig. 3



## ELEMENT HAVING BIMETAL PROPERTIES

## BACKGROUND OF THE INVENTION

The invention relates to an element having bimetal properties which can be used in place of the known bimetal elements for temperature-dependent regulation or control functions or for the indication of temperature.

Bimetal elements are known in a very wide variety of forms for use in indicating temperature and in initiating control operations in dependence upon temperature. These bimetal elements consist of at least two different inseparably connected layers of metal or non-metallic material having different coefficients of thermal expansion. Since, when heated, one of the layers expands to a greater extent than the other, bimetallic elements of this kind bend on a change of temperature, the extent of bending being dependent upon the difference in the coefficients of thermal expansion of the material of the individual layers.

Bimetallic elements can be used in either of two ways: their free unrestricted deflection, dependent upon temperature, may be used such as in bimetal spiral thermometers, or thermal power may be produced by largely completely suppressing the deflection of the element such power doing mechanical work and displacing regulating elements (e.g. bimetal ignition means in gas-heated equipment).

The known forms of bimetallic elements mainly consist of materials having different coefficients of thermal expansion secured together by welding, soldering, bonding and the like.

The known bimetallic elements do not fulfil all the important practical requirements. A particular disadvantage resides in the fact that with relatively broad bimetal strips the isotropy of the thermal expansion results in a very undesirable transverse curvature in addition to the required longitudinal bending, and this transverse curvature leads to mechanical stiffening of the strip. In this way, the required deflection is partly inhibited. In the known forms of bimetallic elements, which are based mainly on combinations of iron-nickel alloys, the choice of material is primarily determined by the thermal properties of the connected layers. This of necessity means that disadvantageous properties as regards electrical conductivity, corrosion-resistance etc., have to be accepted.

## SUMMARY OF THE INVENTION

An object of the present invention is to eliminate the above-stated disadvantages and to provide a bimetal element which possesses particularly advantageous properties. The invention is mainly characterized in that the element is made of a composite fiber material comprising at least one metallic component. Composite fiber materials of this kind contain randomly or specifically distributed fibers embedded in a matrix material, and in a preferred form, both the matrix material and the fibers are made of metallic materials. The composite fiber material can be produced by known metallurgical methods, based for example on powder metallurgy, but it is advantageously produced by jointly cold-shaping the matrix and fiber materials. The term "composite fiber material" is not, however, intended to be limited exclusively to purely metallic combinations in the present case, since for specific uses composite fiber

materials of which the matrix or fiber material is non-metallic, e.g. plastics material, can be produced.

To achieve the bimetal properties in an element in which the composite fiber material comprises a first component constituted by a matrix material and a second component constituted by at least one group of fibers embedded in the matrix material, it is advantageous that there is a coefficient of thermal expansion difference between the first and second components and/or between groups of fibers of the second component. Thus it is advantageous if the coefficients of thermal expansion of at least two groups of fibers embedded in the matrix material of the composite fiber material differ from each other, or if a matrix material is selected that has a coefficient of thermal expansion differing from that of at least one group of fibers embedded in the matrix material. These two possible methods may be combined with each other.

Where the bimetallic effect results from the differing coefficients of thermal expansion of embedded groups of fibers, the matrix material can be freely selected to meet particular additional requirements, namely, corrosion-resistance, specific weight, electrical and thermal conductivity, good mechanical deformability etc.

Similarly, the fibers can be selected not only with the required coefficients of thermal expansion in mind, but also with a view to obtaining the necessary mechanical properties, electrical resistance, magnetic properties and so on. Use may also be made of combinations of materials as normally employed in the known bimetal elements. A considerable advantage of the element of the invention resides in the fact that the matrix material may be selected largely independently of the choice of the fiber that result in deflection of the element under the effect of heat. Furthermore, elements made of a composite fiber material do not become rigid, due to the isotropy of the thermal expansion, as do the known elements in the form of strips. The elements of the invention provide large deflections and large return forces.

In accordance with a further advantageous feature of the invention, the entire cross-sectional area of a group of fibers having a low coefficient of thermal expansion may be greater than the entire cross-sectional area of a group of fibers having a higher coefficient of thermal expansion, since generally the selected matrix material reinforces the expansion of the group of fibers having the higher coefficient.

Groups of fibers can be distributed in the matrix material in various ways and in accordance with the required deflectional movement. In one advantageous form, the groups of fibers can be arranged in parallel layers; this arrangement appears to be particularly suitable in the case of elements in the form of strips. On the other hand, the use of the composite fiber material offers the possibility of making a torsional bimetal element in the form of a strip, this being achieved by arranging a group or groups of fibers over the cross-section of the matrix material in such a way that a temperature-responsive torsional moment results. In this connection, an asymmetric distribution of the groups of fibers in an element in the form of a strip is expedient, so that corresponding torsional moments can be obtained.

A further important improvement may be achieved by embedding, in the element, insulated fibers for electrical heating purposes and/or for conducting current.

By incorporating heating fibers or by appropriately selecting the fibers forming the fiber material, e.g., using the known nickel-iron alloys, which exhibit advantageous coefficients of thermal expansion as well as good electrical resistance properties, a thermoelectric, directly heatable control element can be formed in a simple manner.

The elements may be produced with a wide variety of cross-sectional forms having cornered and circular contours. Also, the dimensions of the elements can be suited to meet particular requirements.

#### BRIEF DESCRIPTION OF THE DRAWINGS

Examples of elements having bimetal properties in accordance with the invention are illustrated in the accompanying drawings in which:

FIG. 1 is a perspective view of a sectioned element in which groups of fibers are distributed in parallel layers;

FIG. 2 shows an element having torsional properties, and

FIG. 3 shows an element in which there are groups of fibers having different cross-sectional dimensions.

#### DETAILED DESCRIPTION OF THE INVENTION

FIG. 1 shows an element in the form of a strip and made of metallic matrix material 1 in which are embedded a first group 3 of metallic fibers having a low coefficient of thermal expansion and a second group 2 of metallic fibers having a higher coefficient of thermal expansion. When the element is heated, the strip acquires a convex upward curvature.

In the example illustrated in FIG. 2, the group of fibers 3 having the lower coefficient of thermal expansion is asymmetrically arranged in relation to the group 2 having the higher coefficient of thermal expansion so as to produce a torsional moment. When the element is appropriately heated, the strip 1 of matrix material twists about its longitudinal axis, so that direct rotary movements can be initiated in a particularly advantageous manner.

In the form shown in FIG. 3, the matrix material 1 is so selected that it reinforces the expansion of the second group 2 of fibers having the higher coefficient of thermal expansion, and it will be seen that the cross-sectional distribution of the fibers of group 3 differs from that of the fibers of group 2. Also in this form insulated resistance-heating wires 4 are embedded between the two groups of fibers so that the strip-like element can be directly heated.

We claim:

1. A composite element having bimetallic properties and comprising:  
5 a first component comprising a matrix material and having imbedded therein at least one additional component, each of said at least one additional components comprising a group of fibers; at least one of said components being metal; and one of said components having a coefficient of thermal expansion different from that of at least another of said components.
2. An element as claimed in claim 1, wherein said at least one additional component comprises a single 10 group of fibers, and wherein said matrix material has a coefficient of thermal expansion different from that of said single group of fibers.
3. An element as claimed in claim 1, wherein said at least one additional component comprises second and third additional components, each of said second and third components comprising a group of fibers.
- 15 20 4. An element as claimed in claim 3, wherein said matrix material has a coefficient of thermal expansion different from that of one of said groups of fibers.
5. An element as claimed in claim 3, wherein the 25 group of fibers of said second component has a coefficient of thermal expansion different from that of the group of fibers of said third component.
6. An element as claimed in claim 5, wherein the 30 total cross-sectional area of the fibers of that group having the lower coefficient of thermal expansion is greater than the total cross-sectional area of the fibers of that group having the higher coefficient of thermal expansion.
7. An element as claimed in claim 5, wherein said 35 groups of fibers of said second and third components are arranged in separate layers in said matrix material, said layers being parallel.
8. An element as claimed in claim 5, wherein said 40 group of fibers of said second component are imbedded in said matrix material asymmetrically of said group of fibers of said third component, whereby a temperature responsive torsional moment is created in said element.
9. An element as claimed in claim 1, further comprising 45 electrically conductive fibers imbedded in said matrix material.
10. An element as claimed in claim 9, wherein said electrically conductive fibers form resistance heating elements.